

1

3,464,886

**DAS-TRIAZINE BRIGHTENERS AND PAPER  
MADE THEREWITH**

Albert Peter Paul, Teaneck, N.J., assignor to American Cyanamid Company, Stamford, Conn., a corporation of Maine  
No Drawing. Filed Apr. 29, 1966, Ser. No. 546,166  
Int. Cl. D21h 3/80

U.S. CL. 162—162

8 Claims

**ABSTRACT OF THE DISCLOSURE**

New non-yellowing brighteners derived from 4,4'-bis(triazinylamino)-stilbene-2,2'-disulfonic acid and which contain as a substituent of the s-triazine ring at least one bis(2-carbamoyethyl) amino moiety are valuable for whitening paper made from cellulosic fibers.

This invention relates generally to new brighteners or optical bleaching agents for paper and to an improved method for whitening paper by the use therewith during some stage of its manufacture, and more particularly, it relates to novel, selected bis-triazinylamino-stilbene compounds containing at least one iminobispropionamide radical (or bis-(2-carbamoyethyl) amino group).

The compounds of this invention which have been found to be especially useful as paper brighteners, have the general formula:



wherein R is a member selected from the group consisting of methoxy and R' as defined hereinafter, and R' is a bis(2-carbamoyethyl) amino group. It is also contemplated that the mono and dialkali metal, ammonium and amine salts of the compounds having the foregoing generalized formula can be used in the formulations for paper brighteners in accord with the invention.

In the past, various chemical compounds have been used as optical bleaching agents and certain optical bleaching agents of the triazinyl stilbene type have been reported in the art as brighteners for paper. However, these prior art compounds have one or more of the following deficiencies:

(1) Some brighteners discolor the paper in the concentration in which they must be present in the paper to be effective.

(2) Some compounds have little or no affinity for cellulose of the paper, that is, they are not substantive.

(3) Others have too much affinity; exhaust too fast thus producing feathering; they are, in effect, too substantive.

(4) Some have insufficient or weak fluorescence when applied in or on paper.

(5) Some fluoresce too green a blue, thus giving a more pronounced yellow effect to the untreated paper which is naturally yellowish.

(6) Some make paper yellow under the acid conditions involved in treatment or in the paper manufacture. They may actually dye paper yellow at low pH.

(7) Some lack usefulness over a wide range of pH from 4 to 9. This may be due to various factors such as lack of stability, quenching of fluorescence, or yellowing, feathering and the like.

(8) Some do not have equal performance in both beater and finishing operations.

2

(9) Some exhibit fluorescence quenching in the presence of alum.

(10) Some are incompatible with other paper additives, fillers, resins and softeners ordinarily used in paper manufacturing.

(11) Finally, the prospective brighteners may have other physical deficiencies such as poor solubility or dispersibility and the like, tending to cause feathering and so forth.

10 It is an object of this invention to provide a new limited group of substituted triazine compounds especially adapted for use as paper brighteners which do not have the above listed deficiencies.

15 It is another object to provide processes for applying these brighteners to give paper an improved chroma and brightness effects.

Other objects will become apparent from the more complete description of the invention presented herein-after.

20 The brighteners of this invention are an improvement over brighteners of related types previously known in the art in that they give distinctive reddish-blue shades of fluorescence which makes paper appear much whiter. They are strongly fluorescent and give a strong clear

25 whitening effect when applied to cellulose materials and especially when used in connection with paper. They are soluble and stable under acid conditions and can be used throughout the pH range which is standard for paper manufacture. They are especially good at low pH where some other brighteners either break down or show reduced efficacy. They have affinity for cellulose and are non-yellowing and non-feathering. They are compatible with other paper chemicals, rosin, alum, fillers, softeners, wet strength resins, dyes and the like. They can also be used to brighten or intensify the color of dyed papers.

30 These compounds are useful for whitening paper when applied to paper pulp during beater operations and in finishing by tub sizing using a size press or by calendering or coating.

35 40 The new compounds or brighteners which are the subject matter of this invention can be prepared by reacting in any order of succession, 2 moles of cyanuric chloride with 2 moles of methanol, 1 mole of 4,4'-diamino-stilbene-2,2'-disulfonic acid or a salt thereof, and 2 moles of an iminobis-propionamide salt. Alternatively, to obtain the species containing two bis(2-carbamoyethyl) amino groups, 2 moles of cyanuric chloride are reacted with 1 mole of 4,4'-diaminostilbene-2,2'-disulfonic acid or a salt thereof and 4 moles of an iminobispropionamide salt. Preferably, the methanol, if used, should be allowed to react first.

45 50 In a typical preferred method for preparation, 2 moles of cyanuric chloride are reacted with 2 moles of methanol in the presence of sodium bicarbonate at a temperature of from about 10° C. to ambient temperatures. The reaction product is then further reacted with approximately 1 mole of 4,4'-diaminostilbene-2,2'-disulfonic acid in solution at 35-50° C., in the presence of sodium hydroxide. Then a solution of 2 moles of iminobispropion-

60 65 amide sulfate is reacted with the last chloro group of cyanuric chloride, in the presence of sodium hydroxide at 50 to 100° C. The whole is then made slightly alkaline. This mixture may be used as a concentrated solution of brightener directly in paper manufacture, or the product may be isolated as the sodium salt, by evaporation or salting out of the product as desired.

70 75 In the preferred practice of this invention, the whitening of paper may be achieved by using 0.01 to 2% of the brightener by weight of the paper or paper pulp, but either smaller or greater concentrations may be used to give corresponding lesser or greater brightening effects as desired.

When the brighteners are used in beater application, a good white is obtained with 0.08-0.5% of brightener by weight of paper pulp. These novel brighteners can be added before or after the alum. They are compatible with wood rosins, fillers, such as titanium dioxide, barium sulfate, zinc sulfide, calcium carbonate, silicon dioxide, starches and clay, with wet strength resins, or with softeners and dyes. Adjustment of the pH is made with alum normally used on the basis of about 4% by weight of the paper. In conventional practice, the pH of the paper pulp mixture is adjusted to 7, or below, before the paper is formed and finished.

The brighteners of this invention may also be used in sizing operations of the paper, such as tub size or size press, in which they may be employed in starch solutions 15 in 0.5-1% concentration or in other aqueous sizing formulations.

The brighteners of this invention may be used in calendering with just the brightener present in water in a concentration of 0.05 to 1% or more. By this method, the 20 completed paper is treated with the solution of brightener to produce a clear white paper.

Further, the brighteners of this invention may be used in coating paper in the usual aqueous coating formulations which include clay-casein, clay-starch or clay-casein-starch. In such coatings, the concentration of brightener may be 0.05-0.3% on the weight of the solids (clay, etc.).

These new brighteners may be used separately or in admixture with other materials for superior whitening of paper in all stages of its manufacture. They have thus 30 been found to be very versatile in their modes of use and application.

The new brighteners of this invention may be converted to methyloated reactive brighteners which can react with cellulose fibers including cotton and paper, as well as other fibers having reactive hydrogen, such as silk, wool and nylon.

The brighteners are methyloated in aqueous solution with at least two moles of formaldehyde for each mole of iminobispropionamide group at temperatures of 20-90° C., and a pH above neutrality, about pH 7.2 to 10, until methylation is complete. Such methylo groups remain 40 active if further methylated or acetylated.

The methyloated brightener may be applied from an aqueous pad bath at pH 4-7 containing an acid catalyst, such as magnesium or ammonium chloride, ammonium sulfate or triethanolamine hydrochloride, in an amount 10-40% by weight of the brightener. The fabric thus padded is dried and cured at 300-375° F. until fixation of the dye to the fabric is complete. The fabric is then soaped, rinsed and dried. The brightener is thus chemically linked to the fiber molecules of the fabric. The fabric is brightened.

The following examples illustrate this invention. They represent, however, only specific illustrative embodiments of the invention, and it is in no way intended to limit the invention thereto.

#### EXAMPLE 1



To a mixture of 18.5 g. (0.1 mole) of cyanuric chloride in 150 ml. acetone, 50 ml. methanol and 2.5 ml. water, is added, with stirring, 16.9 g. (0.20 mole) sodium bicarbonate. The mixture is stirred and heated at 25-35° C. for one hour. To it is added a warm solution of 18.9 g. (0.05 mole) of 97.7% real, technical grade 4,4'-diamino-stilbene-2,2'-disulfonic acid in a mixture of 200 ml. acetone, 200 ml. water and 20 ml. 5 N sodium hydroxide solution. The whole mixture is heated to 50° C., and stirred at 50° C. until a test for free amine is negative.

To this mixture containing 4,4'-bis(4-chloro-6-methoxy-triazin-2-ylamino)stilbene-2,2'-disulfonic acid is added a solution prepared by mixing 25.7 g. (0.10 mole) of iminobispropionamide sulfate with 150 ml. water and 40 ml. 5 N sodium hydroxide solution (0.20 mole). The whole is heated, with stirring to 75° C. (reflux), and held at reflux for two hours. At the end of each hour of the two-hour period, is added 20 ml. 5 N sodium hydroxide solution.

The mixture is cooled, the product filtered and washed with 10% sodium chloride solution and dried in vacuo. Yield 34.8 g. Its absorptivity at 347 m $\mu$  is  $k=48.4$ .

#### EXAMPLE 2



To a mixture of 9.30 g. (0.025 mole) of 99.5% 4,4'-diamino-stilbene disulfonic acid, 150 ml. water, and 50 ml. acetone, there is added, with warming and stirring, 10 ml. (0.05 mole) 5 N sodium hydroxide. The resulting solution is then cooled to 0° C., and a cold solution of 9.23 g. (0.05 mole) cyanuric chloride in 125 ml. acetone added. After stirring 10 minutes at 0-5° C., the pH is adjusted to about 5 with 16 ml. (0.05 mole) 5 N sodium hydroxide solution. There is then added a solution of 25.73 g. (0.10 mole) of iminobispropionamide sulfate, NH(CH<sub>2</sub>CH<sub>2</sub>CONH<sub>2</sub>)<sub>2</sub>H<sub>2</sub>SO<sub>4</sub>, in 100 ml. water and 20 ml. (0.1 mole) 5 N sodium hydroxide solution. The reaction mixture is heated gradually to 70° C. to strip off the acetone, after which the pH is adjusted to about 5 with 5 N sodium hydroxide solution. The mixture is heated to 90° C. and held at 90° C. for one hour. A solution of 5 N sodium hydroxide solution is then added to make the mixture strongly basic. The whole is then cooled and the product filtered. The product is slurried in acetone, filtered, washed with acetone and dried in vacuo over potassium hydroxide. The yield is 20.72 g. of product. Its absorptivity at 348 m $\mu$  is  $k=45.8$ .

#### EXAMPLE 3

##### Beater dyeing of paper pulp

To 4 g. bleached sulfite paper pulp in 100 ml. water is added 0.5 ml. of a 4% solution of alum. The pH is adjusted to 4.5 with 4% alum solution, if necessary.

An 0.1% solution of the brightener is added as follows, 50 based on the absorptivity ( $k$ ) values of the products of Examples 1 and 2, respectively: (a) 3.3 ml. of a 0.1% solution of the product of Example 1 or (b) 3.5 ml. of a 0.1% solution of the product of Example 2.

The whole is stirred 10 minutes. To it is added 1.0 ml. 55 of a 4% solution of light wood rosin followed by stirring for 10 minutes. The pH is readjusted to 4.5 with 4% alum solution (about 1 ml.) and stirring continued for ten minutes.

The pulp mixture is formed into a sheet on a Williams 60 mold, using water adjusted to pH 4.5. The sheet is pressed at 18-20 lb. per square inch, for 30 seconds. It is dried on a drum dryer at 230-240° F., for 5 minutes and conditioned at least 30 minutes at ambient humidity.

Each sheet is observed under ultraviolet light, (U.V. 65 light) and the amount of fluorescence and chroma noted. The compounds of Examples 1 and 2 both show strong blue-white fluorescence compared to little or no fluorescence of untreated paper. In addition, both show good chroma.

Each sheet is then observed under north daylight. Under such light a hue difference is discernible to the trained eye. The sheet of Example 1 is redder than the sheet of Example 2. Both brighteners are redder than the brighteners of the art shown in Table I below. This redness is especially desirable in paper. Both sheets show a

